

Patented May 24, 1927.

1,629,770

# UNITED STATES PATENT OFFICE.

JOHN C. WATSON, OF ATTLEBORO, MASSACHUSETTS, ASSIGNOR OF ONE-HALF TO  
THAYER P. GATES, OF PROVIDENCE, RHODE ISLAND.

## CROSS-DYEING CELLULOSE FABRIC.

No Drawing.

Application filed July 20, 1926. Serial No. 123,803.

My invention relates to an improved process of manufacturing an all cellulose textile fabric in contrasting colors. I employ the words "cellulose textile fabric" to include an all cotton fabric, or a fabric made from the type of rayons which contain substantially the same percentage of cellulose as cotton or a greater percentage of cellulose and which have substantially the same affinity 5 for the same type of dyestuffs as cotton namely, viscose, rayon, cupra-ammonium rayon and chardonet rayon, etc., entirely or mixed with cotton. An application Serial No. 123,801 is filed of even date herewith 10 which is a continuation in part of application #73,471, filed Dec. 5, 1925, which discloses broadly the same invention as this application. There is filed of even date herewith a second application Serial No. 103,802, 15 a continuation in part of application #94-089, filed Mar. 11, 1926, covering specifically a second species of the broad invention disclosed in this application Serial #123,801, filed July 20, 1926. This application covers 20 a third species of the invention.

Hitherto where it has been desired to produce a fabric having a two color effect, either the warp or the filling have been woven of two different materials such as cotton and 30 silk which will take the dye in different shades or amounts, or the warp or filling yarns have had to be separately dyed with two different colors prior to weaving.

The main feature of my process is to treat 35 the warp during the slashing process with the first step of a two step dyeing process, the nature of the ingredient thereof added to the size being such that will have no appreciable effect upon the functioning of the 40 size, nor will the size have any appreciable effect upon its functioning weaving the cloth in the usual manner with a filling and later treating the fabric with the second step of a two step dyeing process, which acts upon the 45 prepared warp to form the dye thereon. I am aware that hitherto it has been suggested to add a direct or substantive dye to the size to simultaneously size and dye the fabric with a one step dyeing process. As 50 the actual water soluble dye has to be inserted with the size it is obvious that in a short space of time, the size bath will become messy and the dyeing irregular and in addition a fast color is not produced. Vari-

ous types of two step dyeing processes are 55 known and it is immaterial for the purposes of my invention what type of a two step dyeing process be employed so long as one is chosen wherein the first step has no appreciable effect upon the functioning of the 60 size, nor the size on its functioning. The types of two step dyeing processes however, may be generally classed as three namely, (A) where the first step thereof consists of 65 treating the warp with a water soluble chemical having non-dyeing properties, such as an organic or inorganic mordant or a soluble mineral salt as described in my application Ser. No. 123,801 and the second step 70 treating it with a dye. (B) Where the first step consists of treating it with a dye or a dye component and the second step consists of treating it with an additional dye component and (C) where the first step consists of treating the warp with a dyestuff in 75 a true or modified form and the second step consists of treating it with a chemical having an oxidizing or reducing action. The subject matter of species C is specifically 80 claimed in this application, namely, where a dyestuff in a true or modified form is inserted with the size and a chemical having an oxidizing or reducing action applied to the entire fabric to combine only with the 85 treated warp.

I am aware that cotton goods of contrasting colors have been made by treating the warp or the filling threads entirely independently of slashing process with a tannin mordant before weaving the cloth in the 90 usual manner with an unprepared filling and then dyeing the fabric with a basic color which acts upon the mordanted warp alone and later dyeing the filling. This process is impractical and expensive for two reasons: 95 It requires the extra cost of an entirely distinct and separate step namely independently of any sizing and prior to weaving of suitably treating the proper threads with a mordant or other first step of a two step dyeing process. Thus the added cost of this added step makes this method of dyeing impractical. The warp is first beamed 100 in a suitable fashion for use in a loom and then passed through a slasher box to cover it with a size so that the individual warp threads will stand up during the friction and wear they receive in the weaving proc- 105

ess, the fabric is then woven in the usual manner. Thus in the usual grey cloth manufacturing plants at present there is no suitable dyeing or mordanting apparatus for 5 performing this separate step. Employing my process however, which merely consists in putting a small amount of the ingredient of the first step of a two step dyeing process right into the slasher a piece of standard 10 equipment in every cotton mill, it is obvious that my process can be employed without the necessity of purchasing extra dyeing or mordanting equipment or without turning the cotton mill into a dye house. After 15 weaving the fabric in the grey form it may then be sent to the dye house where the rest of my process may be completed to dye the fabric in contrasting colors with the usual dyeing equipment by any of the well-known 20 processes.

These and such other objects of my invention as may hereinafter appear will be best understood from a description of various embodiments of my process.

25 My invention includes simultaneously treating the warp threads in the slashing process with a suitable size for weaving and with a first ingredient of a two step dyeing process, each of which has no appreciable effect on the functioning of the other, weaving the cloth in the usual manner with a filling and then treating the entire fabric with the second step of a two step dyeing process which acts upon the prepared warp 30 to impregnate the dye thereon. If desired the filling may be left white or it may also be dyed by again dyeing the fabric with a dye of a different nature and color, which acts on the filling to dye it a contrasting 35 color to the warp. Whether the filling be left white or redyed it is obvious that it will always be of a contrasting color to the dyed warp.

40 It is obvious however that a two step dyeing process may be selected wherein the first step thereof normally comprises treating the warp not with a water soluble chemical having non-dyeing properties, but with a real dye ingredient or a dyestuff in a true or modified form or an intermediate dye component, which would have no appreciable effect on the size, nor the size on its functioning. So far as I am aware no one has hitherto conceived of manufacturing an all cellulose textile fabric having component sets 45 of warp and filling threads of contrasting colors by treating before weaving one of said component sets of threads with a dye ingredient of a two step dyeing process at any 50 stage in the preparation of said set, then weaving said component set with the other component set to form the cloth and then impregnating the dyestuff on the prepared component set by treating the fabric with 55 the second step of the two step dyeing proc-

ess, which acts upon the prepared component set to impregnate the dye thereon. The other component set may be either left white in a contrasting color to the dyed component set or dyed in a contrasting color by again 60 separately dyeing the fabric with a dye of a different nature and color which acts on the unprepared set to dye it a contrasting color to the prepared component set. If desired each component set may be treated with a 65 different dye ingredient of a two step dyeing process and the entire fabric subjected to a second common step of the two step dyeing process, which will simultaneously impregnate each component set with a different dye- 70 stuff. It is thus obvious that the other component set normally the one not sized may be either first dyed or prepared for simultaneously forming the dyestuff thereon with the other component set after weaving or left 75 unprepared. My invention is peculiarly adapted to dye the warp threads with a relatively fast color and specifically includes simultaneously treating the warp threads 80 with a size in the slashing process and simultaneously treating them with a dye ingredient of a two step dyeing process in the 85 same solution. This eliminates the extra cost of an entirely distinct and separate step, namely independently of any sizing and 90 prior to weaving of suitably treating the proper threads with its added cost. At present in the composite process five steps are 95 necessary.

(1) To size the wrap. 100  
(2) To treat the warp threads with a dye ingredient of a two step dyeing process.  
(3) To treat the warp threads with the second step of a two step dyeing process.  
(4) To treat the filling threads with a dye 105 ingredient of a two step dyeing process.  
(5) To treat the filling threads with the second step of a two step dyeing process. 110  
Employing my invention however, where indigosols later to be described are employed it is obvious that these five steps may be cut down to three, namely, step one of sizing the warp threads and step two of treating the warp threads with a dye ingredient of a two step dyeing process may be done simultaneously. Step four of treating the filling threads with a dye ingredient of a two step dyeing process will have to be done separately as usual. The sized and prepared warp threads and the prepared filling threads may be then woven and step three namely, treating the warp threads with the second step of their respective two step dyeing process and in addition step five of treating the filling threads with their respective two step dyeing process may be done simultaneously by treating the warp and the filling threads 115 in the fabric with the same step. 120  
125 This class of a two step dyeing process, namely where the first step in the two step

130

dyeing process comprises treating the material to be dyed with a dye or dye ingredient divides itself into two general classes namely,

5 (B) Where the second step comprises treating the fabric with an additional dye or a dye component and,

(C) Where the second step in the dyeing comprises treating the material desired to 10 be dyed with a chemical having an oxidizing or reducing action to form the dyestuff on the fabric.

I will now describe in detail various embodiments of these different classes, this 15 entire generic class being claimed in application Serial #123,802 filing date July 20, 1926 signed of even date herewith, a continuation in part of application #94,089, filed March 11, 1926, which specifically claims 20 dyestuffs of the generic sub-class B heretofore referred to. Dyeing with a type of dyestuff hereinafter referred to in sub-class C is specifically claimed in this application.

Although as stated, the preparation of 25 either or both of these sets of component threads by treating them with a dye ingredient of a two step dyeing process may be done at any point in the preparation prior to weaving, I preferably so treat the warp 30 threads while slashing and I will specifically describe this treatment in this description of the application of the following dyes. As stated however, it is immaterial whether the filling be first dyed, separately prepared by 35 treating it with a dye ingredient of a two step dyeing process or left unprepared.

I will now specifically describe the application of class C of the two step dyeing process where the first step of a two step 40 dyeing process comprises treating the fabric with a dyestuff modified or unmodified and the second step thereof comprises after treating the fabric with a chemical having an oxidizing or reducing action as specifically 45 claimed in this application. The most important type of dyestuffs of this class includes vat dyestuffs or their derivatives which as is well-known are among the fastest colors. Any suitable type of vat dye- 50 stuffs may be employed. If the vat dyestuff be insoluble it may be adhered to the prepared warp with the size and when the fabric is suitable aftertreated after weaving, the insoluble vat dyestuff will change into 55 a leuco compound to dye the warp on withdrawal from the bath.

Perhaps the most important class of modified dyes which may be dyed in this manner are the stabilized water soluble derivatives 60 of vat dyestuffs which have recently come on the market. Any suitable type of this general type of dyestuff may be employed. What I preferably employ are the types of dyestuffs described in U. S. Patents Nos. 65 1,448,251, and 1,575,958 which are the water

soluble ester-like derivatives of the leuco compounds of any suitable type of vat dyestuffs whether they be produced from indigo as are the types now being put on the market by Société Durand & Huguenin S. A. 70 or those derived from indanthrenes, which according to an article in "The Journal of Dyers and Colorists" for Feb. 1925 are now being put on the market by the Scottish Dyes Ltd. This class of ester-like derivatives whether they be produced from indigo or from indanthrenes or from any other vat dyestuffs are aftertreated to develop the dyestuff on the fabric by reforming the dye by the action of a suitable oxidizing agent. 75 For the purposes of my invention however, any suitable type of a stabilized water soluble derivative of a vat dyestuff may be employed like the dehydro-indigos as described in German Patents Nos. 217,477—220,173— 80 237,262—239,314 which are later developed on the fabric by reforming the dye by the action of a suitable reducing agent.

I will specifically describe the application of an indigosol, such as indigosol O. B. 90 for blue sold in America by the General Dyestuffs Corporation, specifically applying it to the warp in the slashing process. The slasher tank solution may be prepared as follows: 25 pounds of sago or other suitable 95 size are added to 50 gallons of water. To this bath is also added as the dye ingredient of the two step dyeing process 1-3 pounds of indigosol blue O 4 B the amount depending on the shade desired, preferably previously dissolved in about 3 gallons of water. These materials may then be boiled together for about 20 minutes in the size tank after which an amount of sodium nitrite equal in weight to the indigosol used is added. After the contents have been 100 mixed well they are then run into the slasher box and the warp sized as usual. It is thus obvious that the goods may be prepared for dyeing the warp with a vat color 105 by adding a small proportion of a vat dyestuff, modified, or unmodified to the sizing mixture. In place of sago, potato, corn, or any other suitable starch, flour or any other suitable sizing material may be employed. 110 and in place of indigosol O 4 B any type of vat dyestuff modified or unmodified preferably a stabilized water soluble ester-like derivative of the leuco compound may be employed. In place of sodium nitrite any 115 suitable oxidizing agent may be employed, or if desired this may be dispensed with. The goods are then woven as hitherto explained and then sent from the weave shop to the dye house.

After weaving, the dyestuff is developed on the warp by suitably forming the dye thereon by any suitable aftertreatment depending on the nature of the vat dyestuff employed. Where an indigosol or any 120 125 130

water soluble ester-like derivative of a vat dyestuff has been employed as the first dye ingredient, I preferably reform the dyestuff on the warp by an action of a suitable oxidizing agent. Although this may be done in any suitable manner, it is preferably done by passing the woven fabric through a jig. To reform the dyestuff by oxidation and to free the oxygen from the sodium nitrite 10 preferably added to the first dye ingredient with the size, I preferably fill the jig with a 2° Tw. sulphuric acid, when dyeing with an indigosol or like ester-like derivative the color will immediately be developed on the 15 warp. If other types of vat dyestuffs or their stabilized water soluble derivatives be employed they may be suitably reduced to the desired leuco compound in any well-known manner, after which the dyestuff will 20 be reformed on the fabric by oxidation on exposure to the air. Any suitable type of acid may be employed and any other suitable type of an oxidizing agent other than nitrite of soda may be employed. The 25 goods are then washed, soaked and washed, preferably in a jig or if desired dried and mercerized. If not mercerized after the last wash the goods may be re-dyed in the same 30 jig, preferably with a three or four per cent solution of a substantive or direct color of a different shade. After this they may be washed, dried and finished in the usual manner. If it is desired to have the filling 35 threads un-dyed and left a white in a contrasting color to the dyed warp the last step of dyeing the fabric with a direct color may be dispensed with. If it is desired to dye the filling threads a faster color then they 40 may be dyed with a direct color in a contrasting shade, it is obvious that the filling threads may also prior to weaving be similarly treated with a different type of indigosol such as indigosol helio. The fabric is woven in the usual manner and latter on 45 passing the fabric through acid, a blue dyestuff will be developed on the warp and a helio dyestuff will be dyed on the filling, thus as explained eliminating two of the five steps hitherto necessary in dyeing of this 50 description.

It is obvious that by simultaneously treating the warp in the slasher box with a size and with a first step of a two step dyeing process, each of which has no appreciable 55 effect on the functioning of the other, weaving the cloth in the usual manner with the filling and treating the fabric with the second step of a two step dyeing process, which acts on the prepared warp to form the dye 60 thereon, that it reduces the cost of manufacturing an all cellulose textile fabric in contrasting colors by the cost of one entire step in the process, as hitherto explained, namely by the separate step by treating the warp 65 separately with the first step of the two step

dyeing process. It is apparent that I have provided a process which may be readily put in the cotton mills without extra equipment and that I have shown for the first time a method of dyeing cellulose fabrics in 70 contrasting colors with colors faster than any hitherto used for this purpose.

As explained, my invention broadly includes the step in the process of manufacturing an all cellulose textile fabric having 75 component sets of warp and filling threads of contrasting colors, which comprises, treating before weaving one of said component sets of threads with a dye ingredient of a two step dyeing process in any stage in 80 the process of manufacture thereof or both sets with a different dye ingredient of a two step dyeing process. Where this is done other than in the size bath however, it is 85 obvious that the cotton mills will have to be provided with additional tanks or other equipment. Where it is desired to thus treat the warp or the filling threads other than in the slashing process they may be treated in exactly the same fashion as hitherto explained with the same strength solutions omitting the addition of the size to the 90 first step.

It is obvious that in place of treating the entire warp or filling with the first step of a 95 two step dyeing process only parts of them may be so treated and I therefore employ the phrase in the claims "component sets of warp and filling threads" to include the entire warp or filling threads or any desired 100 part thereof. I employ the words "cellulose textile fabric" to include an all cotton fabric, or a fabric made from the type of rayons which contain substantially the same percentage of cellulose and which have substantially the same affinity for the same type of dyestuffs as cotton namely, viscose rayon, cupra-ammonium rayon and chardonet rayon, etc., entirely or mixed with cotton.

I employ the word "weave" in the claims 110 in its broad sense as defined in Webster's Dictionary of 1866 which defines it as follows: 1. "To unite, as threads of any kind, in such a manner as to form a texture; to entwine or interlace into a fabric as to weave 115 wool, silk and the like; hence, to unite by close connection or mixture, to unite intimately . . .

2. To form, as cloth, by interlacing threads; to compose, as a texture of any 120 kind, by putting together textile materials; hence, to form into a fabric; to compose."

It is understood that my invention is not limited to the specific processes described and the various deviations may be made 125 therefrom without departing from the spirit and scope of the appended claims.

What I claim as new and desire to secure by Letters Patent is:

1. The herein described improved process 130

- of manufacturing an all cellulose textile fabric having component sets of warp and filling threads of contrasting colors which comprises treating before weaving one of 5 said component sets with a dyestuff, treating the other component set with a different dyestuff, then weaving said component sets to form the fabric and after weaving treating the fabric with a chemical which acts on 10 one component set to form a dyestuff of one color thereon and acts on the other component set to form a dyestuff of a different contrasting color thereon.
2. The herein described improved process 15 of manufacturing an all cellulose textile fabric in contrasting colors, which comprises simultaneously treating the warp in the slashing process with a size and with a dyestuff, each of which has no appreciable effect 20 on the functioning of the other, treating the filling with a different dyestuff, then weaving said warp and filling in the usual manner to form the fabric and after weaving treating the fabric with a chemical which acts on 25 the warp to form a dyestuff of one color thereon and which acts on the filling to form a dyestuff of a contrasting color thereon.
3. The herein described improved process 30 of manufacturing an all cellulose textile fabric having component sets of warp and filling threads of contrasting colors which comprises treating before weaving one of said component sets with a vat dyestuff, treating the other component set with a different vat 35 dyestuff, then weaving said component sets to form the fabric and after weaving treating the fabric with a chemical which acts on one component set to form a dyestuff of one color thereon and acts on the other component set to form a dyestuff of a different contrasting color thereon.
4. The herein described improved process 40 of manufacturing an all cellulose textile fabric in contrasting colors, which comprises simultaneously treating the warp in the slashing process with a size and with a vat dyestuff, each of which has no appreciable effect on the functioning of the other, treating the filling with a different vat dyestuff, 45 then weaving said warp and filling in the usual manner to form the fabric and after weaving treating the fabric with a chemical, which acts on the warp to form a dyestuff of one color thereon and which acts on the filling to form a dyestuff of a contrasting color thereon.
5. The herein described improved process 50 of manufacturing an all cellulose textile fabric having component sets of warp and filling threads of contrasting colors, which comprises treating before weaving one of said component sets of threads with a stabilized soluble derivative of a vat dyestuff, then weaving said component set with the other 55 component set to form the fabric, aftertreat- ing the fabric to form the vat dyestuff on the prepared component set and again dyeing the fabric with a dye of a different nature and color, which acts on the unprepared component set to dye it a contrasting color 70 to the prepared component set.
6. The herein described improved process 75 of manufacturing an all cellulose textile fabric having component sets of warp and filling threads of contrasting colors, which comprises treating before weaving one of said component sets of threads with a stabilized soluble derivative of a vat dyestuff, then weaving said component set with the other component set to form the fabric, and treat- 80 ing the fabric to form the vat dyestuff on the prepared component set.
7. The herein described improved process 85 of manufacturing an all cellulose textile fabric having component sets of warp and filling threads of contrasting colors which comprises treating before weaving one of said component sets with a stabilized soluble derivative of a vat dyestuff, treating the other component set with a different stabilized soluble derivative of a vat dyestuff, then weaving said component sets to form the fabric and aftertreating the fabric to form a vat dyestuff on one prepared component set and simultaneously impregnate the other 90 component set with a vat dyestuff of a different contrasting color.
8. The herein described improved process 95 of manufacturing an all cellulose textile fabric in contrasting colors, which comprises simultaneously treating the warp in the slashing process with a size and with a stabilized soluble derivative of a vat dyestuff, each of which has no appreciable effect on the functioning of the other, weaving the fabric in 100 the usual manner with a filling, treating the fabric to form the vat dyestuff on the prepared warp and again dyeing the fabric with a dye of a different nature and color which acts upon the unprepared filling to dye it a 105 contrasting color to the warp.
9. The herein described improved process 110 of manufacturing an all cellulose textile fabric in contrasting colors, which comprises simultaneously treating the warp in the slashing process with a size and with a stabilized soluble derivative of a vat dyestuff, each of which has no appreciable effect on the functioning of the other, weaving the fabric in the usual manner with a filling, and 115 treating the fabric to form the vat dyestuff on the prepared warp.
10. The herein described improved process 120 of manufacturing an all cellulose textile fabric in contrasting colors, which comprises simultaneously treating the warp in the slashing process with a size and with a stabilized soluble derivative of a vat dyestuff, each of which has no appreciable effect on the functioning of the other, treating the 125 130

filling with a different stabilized water soluble derivative of a vat dyestuff, then weaving said warp and filling in the usual manner to form the fabric and aftertreating the fabric to simultaneously form a vat dyestuff on the prepared warp and simultaneously impregnate the filling with a vat dyestuff of a different contrasting color.

11. The herein described improved process of manufacturing an all cellulose textile fabric having component sets of warp and filling threads of contrasting colors, which comprises, treating before weaving one of said component sets with a soluble ester-like derivative of a vat dyestuff, then weaving said component set with the other component set to form the fabric and then developing the dye on the prepared component set by reforming the dyestuff by the action of a suitable oxidizing agent on the entire fabric and again dyeing the fabric with a dye of a different nature and color which acts on the unprepared component set to dye it in a contrasting color to the prepared component set.

12. The herein described improved process of manufacturing an all cellulose textile fabric having component sets of warp and filling threads of contrasting colors, which comprises treating before weaving one of said component sets with a soluble ester-like derivative of a vat dyestuff, then weaving said component set with the other component set to form the fabric and then developing the dye on the prepared component set by reforming the dyestuff by the action of a suitable oxidizing agent on the entire fabric.

13. The herein described improved process of manufacturing an all cellulose textile fabric having component sets of warp and filling threads of contrasting colors which comprises treating before weaving one of said component sets with a soluble ester-like derivative of a vat dyestuff, treating the other component set with a different soluble ester-like derivative of a vat dyestuff, then weaving said component sets to form the fabric and then simultaneously developing a dye on one prepared component set and a different dye on the other prepared component set by reforming the dyestuffs by the action of a suitable oxidizing agent on the entire fabric.

14. The herein described improved process of manufacturing an all cellulose textile fabric in contrasting colors, which comprises simultaneously treating the warp in the slashing process with a size and with a soluble ester-like derivative of a vat dyestuff, each of which has no appreciable effect on the functioning of the other, weaving the fabric in the usual manner with a filling, then developing the dye on the prepared warp by reforming the dyestuff by the action of a suitable oxidizing agent on the entire fabric and again dyeing the fabric with a

dye of a different nature and color which acts upon the unprepared filling to dye it a contrasting color to the warp.

15. The herein described improved process of manufacturing an all cellulose textile fabric in contrasting colors, which comprises simultaneously treating the warp in the slashing process with a size and with a soluble ester-like derivative of a vat dyestuff, each of which has no appreciable effect on the functioning of the other, weaving the fabric in the usual manner with a filling and then developing the dye on the prepared warp by reforming the dyestuff by the action of a suitable oxidizing agent on the entire fabric.

16. The herein described improved process of manufacturing an all cellulose textile fabric in contrasting colors, which comprise simultaneously treating the warp in the slashing process with a size and with a soluble ester-like derivative of a vat dyestuff, each of which has no appreciable effect on the functioning of the other, treating the filling with a different soluble ester-like derivative of a vat dyestuff, then weaving said warp and filling in the usual manner to form the fabric and then simultaneously developing the dye on the prepared warp and a different dye on the prepared filling by reforming the dyestuffs by the action of a suitable oxidizing agent on the entire fabric.

17. The herein described improved process of manufacturing an all cellulose textile fabric having component sets of warp and filling threads of contrasting colors which comprises treating before weaving one of said component sets of threads with a soluble ester-like derivative of a vat dyestuff and a potential oxidizing agent, weaving said component set with the other component set to form the fabric and passing the fabric through acid in order to develop the dyestuff upon the prepared component set and again dyeing the fabric with a dye of a different nature and color, which acts on the unprepared component set to dye it in a contrasting color to the prepared component set.

18. The herein described improved process of manufacturing an all cellulose textile fabric having component sets of warp and filling threads of contrasting colors which comprises treating before weaving one of said component sets of threads with a soluble ester-like derivative of a vat dyestuff and a potential oxidizing agent, weaving said component set with the other component set to form the fabric and passing the fabric through acid in order to develop the dyestuff upon the prepared component set.

19. The herein described improved process of manufacturing an all cellulose textile fabric having component sets of warp and filling threads of contrasting colors which comprises treating before weaving one of

said component sets with a soluble ester-like derivative of a vat dyestuff and a potential oxidizing agent, treating the other component set with a different soluble ester-like derivative of a vat dyestuff and a potential oxidizing agent, then weaving said component sets to form the fabric and passing the fabric through acid in order to develop a dyestuff upon one prepared component set and a different dyestuff on the other prepared component set.

20. The herein described improved process of manufacturing an all cellulose textile fabric in contrasting colors, which comprises simultaneously treating the warp in the slashing process with a size and with a soluble ester-like derivative of a vat dyestuff and a potential oxidizing agent, each of which has no appreciable effect on the functioning of the other, weaving the fabric in the usual manner with a filling, and passing the fabric through acid in order to develop a dyestuff upon the prepared warp and again dyeing the fabric with a dye of a different nature and color which acts upon the unprepared filling to dye it a contrasting color to the warp.

21. The herein described improved process of manufacturing an all cellulose textile fabric in contrasting colors, which comprises simultaneously treating the warp in the slashing process with a size and with a soluble ester-like derivative of a vat dyestuff and a potential oxidizing agent, each of which has no appreciable effect on the functioning of the other, weaving the fabric in the usual manner with a filling, and passing the fabric through acid in order to develop a dyestuff upon the prepared warp.

22. The herein described improved process of manufacturing an all cellulose textile fabric in contrasting colors, which comprises simultaneously treating the warp in the slashing process with a size and with a soluble ester-like derivative of a vat dyestuff and a potential oxidizing agent, each of which has no appreciable effect on the functioning of the other, treating the filling with a different soluble ester-like derivative of a vat dyestuff and a potential oxidizing agent, then weaving said warp and filling in the usual manner to form the fabric and passing

the fabric through acid in order to develop a dyestuff upon the prepared warp and a different dyestuff on the prepared filling.

55

23. An all cellulose textile fabric in the gray state made up of component sets of threads interwoven with other component sets of threads, one of said component sets being impregnated with a stabilized soluble derivative of a vat dyestuff and another of said component sets being impregnated with a stabilized soluble derivative of a different vat dyestuff.

60

24. An all cellulose textile fabric in the gray state made up of component sets of threads interwoven with other component sets of threads, one of said component sets of threads being impregnated with a stabilized soluble derivative of a vat dyestuff.

70

25. An all cellulose textile fabric in the gray state made up of component sets of threads interwoven with other component sets of threads, one of said component sets of threads being impregnated with a soluble ester-like derivative of a vat dyestuff and another of said component sets being impregnated with a soluble ester-like derivative of a different vat dyestuff.

75

26. An all cellulose textile fabric in the gray state made up of component sets of threads interwoven with other component sets of threads, one of said component sets of threads being impregnated with a soluble ester-like derivative of a vat dyestuff.

80

27. An all cellulose textile fabric in the gray state made up of component sets of threads interwoven with other component sets of threads, one of said component sets of threads being impregnated with a soluble ester-like derivative of a vat dyestuff and a potential oxidizing agent and another of said component sets being impregnated with a soluble ester-like derivative of a different vat dyestuff and a potential oxidizing agent.

85

28. An all cellulose textile fabric in the gray state made up of component sets of threads interwoven with other component sets of threads, one of said component sets of threads being impregnated with a soluble ester-like derivative of a vat dyestuff and a potential oxidizing agent.

90

In testimony whereof I affix my signature.  
JOHN C. WATSON.